

# UNITED STATES PATENT OFFICE.

CHARLES LEOPOLD BAILLARD, OF ROUEN, DEPARTMENT OF THE SEINE-  
INFÉRIEURE, FRANCE.

## PROCESS OF TREATING MINERAL OILS.

SPECIFICATION forming part of Letters Patent No. 340,411, dated April 20, 1886.  
Application filed December 24, 1885. Serial No. 186,643. (No specimens.)

*To all whom it may concern:*

Be it known that I, CHARLES LEOPOLD BAILLARD, a citizen of France, residing at Rouen, in the Department of the Seine-Inférieure, have invented new and useful Improvements in Treatment of Mineral Oils, of which the following is a specification.

This invention relates to the treatment of mineral oils, particularly those of the formula  $C_nH_{2n+2}$ , for the purpose of rendering them analogous to oils of animal and vegetable origin.

Heretofore the use of mineral oils has been limited, in consequence of their special constitution and certain defects resulting therefrom, so that for many purposes use must be made of animal and vegetable oils, notwithstanding their relatively high price. In particular, mineral oils are unsuited to oiling wool, because it is impossible afterward to remove them, or to the manufacture of soaps, because they will not combine with alkali, or to lubrication, because of their fluidity. I have thought that by oxidizing mineral oils, so as to form bodies analogous to ternary oils of animal or vegetable origin, the result will be to render them soluble in alkalies, (soda, potash, ammonia, &c.,) and that consequently they can be mixed with these alkalies. Mineral oil oxidated in this way could be used for oiling wool, for the manufacture of soap, and for lubrication. My process of oxidation for accomplishing these objects is based upon the fact that the oleic acid of distillation or saponification possesses in a high degree the property of yielding to mineral oils a part of its oxygen, and (a very remarkable thing) that in this connection oleic acid acts the part of a carrier for the oxygen of the air.

My process consists in heating to one hundred and sixty (160) degrees centigrade a mixture of mineral oils and oleic acid. Animal fats in a rancid state act the same part as oleic acid, and so, also, rancid olive-oil, cotton-seed oil, linseed-oil, peanut-oil, castor-oil, and others. The proportion of oleic acid or rancid oils, or fats varies from five to twenty-five per cent. (5% to 25%) of the weight of the mineral oil. They oxidate the latter in proportion to the quantities introduced. It is ad-

vantageous to introduce the mixture into a heater, for mixing the ingredients better together. The temperature of one hundred and sixty (160) degrees centigrade has been used with the best results in most cases; but I have obtained with certain oils a complete oxidation at one hundred and forty (140) degrees centigrade. It is also to be noted that even at lower temperatures the oxidation, commenced but incomplete, continues and is effected by the aid of the oxygen of the air. Fiber can therefore be oiled with oil treated as before described, even below one hundred and forty degrees (140°) centigrade, the oxidation continuing in the cold during spinning and weaving.

For wagon-grease or lubricating material mineral oils treated as described can be combined with soda or potash in quantities sufficient to make a soft soap. When about two to ten per cent. (2% to 10%) in weight of fixed vegetable oils—such as cotton-seed, castor peanut, olive, sesame, colga, linseed, and others—is added to mineral oils treated as above described, the latter become adapted to serve as mordants for dyeing vegetable fiber.

I claim—

1. The process of treating mineral oils of the general formula  $C_nH_{2n+2}$  by oxidating the same, and thereby rendering them analogous to the ternary oils of animal or vegetable origin, and capable of use in place of the same substantially as described.

2. The process of oxidating mineral oils by treating the same with oleic acid of distillation or saponification, or with rancid oil or fat, substantially as described.

3. The described improvement in the art employing oils, whereby the necessity of employing oils of animal or vegetable origin for many purposes is avoided, the said improvement consisting in oxidating mineral oil and applying the oxidated oil in said industry substantially as described.

In testimony whereof I have signed the specification in the presence of two subscribing witnesses.

CHARLES LEOPOLD BAILLARD.

Witnesses:

JULES T. AYOLLET,  
T. CHAUDET.